

Oct. 16, 1934.

E. BUTLER ET AL

1,977,262

## ORE CONDITIONING PROCESS

Filed April 23, 1930



## UNITED STATES PATENT OFFICE

1,977,262

## ORE CONDITIONING PROCESS

Emmett Butler and Arthur K. Knickerbocker,  
St. Paul, and Richard O. Hocking, Nashwauk,  
Minn.; Francis D. Butler special administrator  
of said Arthur K. Knickerbocker, deceased

Application April 23, 1930, Serial No. 446,598

3 Claims. (Cl. 209—2)

The invention relates to the conditioning of ore and more particularly has reference to a process for mechanically separating the ore from the gangue.

- 5 A large proportion of all ore mined contains such a percentage of impurities as to make it unavailable for immediate commercial use. As a result of this condition the art of mineral separation or concentration has, within the last  
10 fifty years, been highly developed. At the present time, ore which was heretofore commercially unavailable, may now be used as a result of special treatment. However, the fact nevertheless remains that a considerable amount of ore  
15 of many minerals is wasted because of the lack of an adequate process for the removal of the impurities contained therein. Particularly is this true of iron ore which frequently contains high percentages of silica.  
20 Within recent years developments in the ore separation art have been directed to improvements of separate process steps and apparatus for carrying out the same so that the maximum yield  
25 of concentrates having low proportions of impurities may be obtained from crude ore. Up to the present it appears that refinements of this nature have reached their ultimate limit. Still the concentrates obtained are not up to the desired standard as they contain high percentages  
30 of undesirable constituents as impurities. The reason for this condition may be found in the economic theory of intensive utilization. Further conditioning of the concentrates so as to reduce the proportion of impurities contained  
35 therein, while often being feasible "on paper" have proved to be impractical in actual practice because they exceed the limit of economical production conditions.

The major object of this invention is the provision of a conditioning process for ore to produce a maximum yield of merchantable concentrates.

An equally important object of the invention is the provision of an ore concentrating method wherein low grade ore may be conditioned so as to remove the maximum amount of impurities therefrom.

Another object of the invention is the provision of a process for conditioning ore in which the oversize from a sizing stage is jigged so as to concentrate the same.

Another object of the invention is to devise an ore conditioning process wherein the fines from the sizing stage are washed and classified, and  
55 the concentrates from the classifying stage sub-

jected to a second washing stage, to produce concentrates for use as a commercial product.

Still another object is the provision of an ore concentrating process whereby the fines from a sizing stage are treated in a log washer, the oversize therefrom being classified and the concentrates from the classifier and log washer being treated in a second washing stage to produce concentrates ready for commercial use.

Yet another object of the invention is the provision of an ore concentrating method in which the crude ore is suitably sized, the oversize therefrom subjected to a jiggling stage, the fines from the sizing stage washed and classified, and the concentrates from the washing stage and the classifying stage subjected to a second washing stage to produce concentrates ready for commercial use.

Still a further object of the invention is the conditioning of ore comprising subjecting the ore to a sizing stage, passing the oversize therefrom to a jiggling stage, crushing the tailings from the jiggling stage and magnetically separating the concentrate therefrom and sintering the same.

Yet a further object of the invention is to devise an ore separation method wherein the ore is subjected to a sizing stage, the fines therefrom washed and classified, the concentrates from the classifying stage subjected to a second washing stage, the tailings from the second washing stage subjected to magnetic separation so as to remove the ore therefrom and then sintering the ore.

With these and other objects in view, the invention consists in the method and apparatus to be hereinafter set forth and claimed with the understanding that the several apparatus features disclosed and the various steps and stages of the process set forth in the procedure may be widely varied without departing from the spirit of the invention or the scope of the appended claims.

The invention comprehends the provision of an ore concentrating or separating process wherein in a great amount of impurities are removed from the ore so that a low grade ore may be converted into a merchantable form. One method of practically effecting the concept of the invention is the provision of a sizing stage wherein the ore may be suitably sized, the oversize being subjected to a jiggling treatment. The fines from the sizing stage may be washed and classified and the concentrates from the washing and/or classifying stage subjected to a second washing

stage so that the resulting concentrates therefrom will be ready for commercial use. The invention further comprehends the treatment of the tailings from the jiggling stage and the second washing stage so that they may be made available.

In order to make the invention more clearly understood there is shown in the accompanying drawing a diagrammatic representation for carrying the same into practical effect. It is to be understood that the various steps of the process are not to be limited to the forms shown in the drawing, which for the purpose of explanation have been made the subject of illustration.

In the drawing:

The figure is a diagrammatic view of a plant layout for carrying out the process forming the subject-matter of this application.

20 In the drawing there is shown a layout or flow sheet for an ore conditioning plant in which the crude ore is first introduced into a grizzly 1 at the head of the plant. Ore of plus 5" in size is deposited in a rock car while the undersize drops into the pocket of the grizzly, and is thence conveyed by a belt conveyor to a trommel 2 which has associated therewith a rock screen 3. Other types of sizing apparatus than a trommel may be employed under certain circumstances.

30 Before entering the trommel the ore may be weighed by means of a weightometer 4. While a weightometer of the Merrick type has been shown, it is to be understood that any other suitable type of weightometer may be employed if desired.

35 The trommel 2 is provided with 1" openings through which the fines of the crude ore pass directly to a second trommel 5. As stated in connection with trommel 2, other sizing apparatus may be employed in lieu of trommel 5.

40 The oversize passes to the rock screen 3, provided with 3½" openings so that only ore under that size may pass therethrough. Ore passing through the mesh of the screen is led to a crusher 6 of the Symons type although any other crusher desired may be employed. Crushed ore from the crusher 6 is led to the second trommel 5 where it is mixed with the fines from the trommel 2. As indicated in the drawing, oversize from the screen 3 associated with the trommel 2 is conducted in any convenient manner to a rock hopper 7.

The grizzly and the trommels 2 and 5, it will be appreciated serve to size the ore preparatory to subsequent treatment to be hereinafter described. 55 It is to be understood, however, that a procedure other than herein set forth may be employed for sizing.

60 The 20 foot trommel 5 is provided with ½" openings although it is to be understood that the invention is not limited to a trommel of this length having openings of this size. For example, if desired ¾" openings in the trommel may be used and other trommel lengths employed.

65 It will be appreciated that in the sizing stage described the ore is progressively reduced in size by separation in the machines or apparatus mentioned.

70 Fines or undersize from the trommel 5 are transported in any convenient manner to a log washer 8 of any suitable type. The log washer may have either a single log or a plurality of logs formed either of wood or metal. At its overflow end the log washer is provided with an overflow line in which the sands and other similar materials of the log washer are conducted to a Dorr

bowl classifier 9 or any other classifier. In the Dorr bowl classifier the ore is further treated and the tailings therefrom are conducted to a tailings pond as indicated or to further treatment.

80 The concentrates from the log washer and the Dorr bowl classifier are usually collected in a concentrate bin 11 after which they are ready for shipment and commercial refining. It is also the custom to mix with these concentrates the oversize from the trommel 5. Instead of employing this practice, however, the invention contemplates further treatment of the concentrates and the oversize just mentioned, so as to remove from them further amounts of impurities, which in the case of iron are principally silica.

85 Table I, which is compiled from data obtained at the Harrison washing plant of Cooley, Minnesota, in the Mesaba iron range, shows an analysis of these concentrates and the oversize. With reference to this table the desirability of further conditioning the ore so that a better commercial product may be obtained is at once appreciated. This table is as follows:

TABLE I  
Ore analysis at the Harrison washing plant

| Stage of treatment                     | Tonnage percentage | Percentage composition of the major constituents of ore |                |
|----------------------------------------|--------------------|---------------------------------------------------------|----------------|
|                                        |                    | Iron                                                    | Silica         |
| ½" trommel oversize.....               | 31.5               | 54.64<br>53.74                                          | 14.85<br>17.05 |
| Logwasher concentrates.....            | 11.0               | 57.50<br>56.43                                          | 12.50<br>14.45 |
| Dorr bowl classifier concentrates..... | 7.50               | 56.25<br>50.55                                          | 15.25<br>20.76 |

While the ore contains other substances such as oxygen, alumina, magnesia, phosphorus, carbon dioxide, sulphur and water, iron and silica are by far the principal constituents. Hence reference is made only to the iron and silica content. It is to be noted that two analyses are given for the ore at the different stages of treatment listed. These refer to the maximum and minimum value of the iron and silica content of the ore. Each value given in the heading "Tonnage percentage" shows the percentage of the total tonnage of crude ore placed in the grizzly at the head of the plant at the particular stage of treatment. For the sake of simplicity consider one hundred tons of crude ore deposited in the grizzly. Ten tons or 10% of the total is removed as rock. Of this 90 tons remaining, 58.5 tons leave the second trommel as fines and 31.5 tons leave as oversize.

115 From the foregoing table the desirability of further separating the silica from the ore so as to obtain a better commercial product is at once apparent. In order to carry this out the oversize from the trommel 5 and the concentrates from the log washer and the Dorr bowl classifier are subjected to separate treatments and the concentrates from these steps are finally combined in 120 the concentrate bin 11.

125 As an example, the oversizes from the trommel 5 may be subjected to a jiggling step although it is to be understood that if the grade warrants it is sometimes desirable to ship these oversizes direct. 130 The oversize from the trommel 5 is conducted to a sizing screen 12 or other appropriate sizing apparatus, located at the head of the jiggling plant. The fines from this sizing screen of less than ¾" are directed to a battery of jigs 13 135

which may be of the McLanahan type while the oversizes from the screen are conducted to similar jigs 14. As is well known the McLanahan jig is of the piston type and is usually provided with four sieves mounted in one tank. While McLanahan jigs have been disclosed in connection with the process it is to be understood that other jigs may be employed if desired. Although the McLanahan jig employs water as a working fluid, it will be appreciated that the use of an air jig would not exceed the spirit of the invention nor depart from the scope of the appended claims.

Tailings from the jigs indicated by 13 and 14 are combined together and are conducted in any desirable manner to a shipping bin or stock pile. The concentrates of the jigs, on the other hand, are sent to the concentrate bin 11 and if desired may be mixed with the concentrates returned from a second washing stage, which will be presently described.

In order to reduce the silica content of the log washer and Dorr bowl concentrates a second washing step is employed. As represented in the drawing, concentrates from the washer 8 and the classifier 9 may pass as indicated by lines 16 and 17 respectively to a second washing stage employing a battery of washing machines of the Rheolaveur type generally designated by the numeral 10.

As is well known the Rheolaveur washing machines are of the shallow pocket launder type classifier, the operation of which depends upon the stratification of the crude material by reason of different specific gravities, in the different rate of movement along the trough of the launder and in the different settling velocity of the different materials. When a mixture of particles is first introduced into troughs, such as those shown, stratification occurs, the heavier materials settling to the bottom and moving at a less rapid rate than the upper materials. Suitable discharge slots are provided, and when reached the heavier material at the bottom of the trough is deposited therein while the lighter material continues along the trough. A suitable rewash line 15 is provided so that the material received in the last launder of the plant may be taken to the head launder and rewashed if desired. The concentrates in this instance, iron ore, are taken off and deposited in a concentrate bin 11. Tailings or the lighter substance contained in the ore, such as the silica are deposited in a tailings pond.

While the concentrates from the log washer and the Dorr bowl classifier have been indicated as passing to the Rheolaveur plant, it is to be understood that the concentrates from either of these stages may be sent directly through line 18 to the concentrate bin if desired. In some instances it may be desirable to send the concentrates of the log washer to the bin 11 and the concentrates from the Dorr bowl classifier to the Rheolaveur machines. On the other hand it may be desirable to direct the log washer concentrates to the Rheolaveur plant and the classifier concentrates to the collecting bin. Likewise it should be understood that the concentrates from the log washer, may if desired, be conducted through line 19 as indicated on the drawing, to the sizing screen 12 and thence to the jigs 13 and 14.

It has been stated that one of the objects of the invention is the conditioning of the tailings from the jigs and from the Rheolaveur machines. From an inspection of Table II, which is compiled from data obtained from the same source

as that disclosed in Table I, it may be observed that the quantity or mass of these tailings represent a relatively large percentage of the total tonnage. Table II is as follows:

TABLE II  
*Analysis of tailings at the Harrison washing plant*

| Stage of treatment        | Tonnage percentage | Percentage composition of the major constituents of the material |                |
|---------------------------|--------------------|------------------------------------------------------------------|----------------|
|                           |                    | Iron                                                             | Silica         |
| Jig tailings.....         | 6.3                | 48.26<br>30.54                                                   | 26.25<br>52.77 |
| Rheo. mach. tailings..... | 3.75               | 52.50<br>44.35                                                   | 20.00<br>29.52 |

(Note: The values given in connection with Table II are composed in a manner similar to that employed in connection with Table I.)

Instead of discarding and wasting these rejects of the jigging and the Rheolaveur washing stage, the present invention contemplates further processing so as to obtain a merchantable product. This is accomplished by first crushing these tailings so as to liberate the mineral from the silica. The size of the crushed material should be within that required for the proper separation of iron and silica and treatment of material by a cylindrical rotating kiln. This type of kiln or any other suitable type desired may be employed. In the kiln the material is preheated so as to drive off all of the moisture contained therein and its temperature is raised to approximately that required for roasting.

After suitable heat treatment in the drier, as described, the ore is passed to a roaster where it is subjected to a temperature of from 300°-700° C. in a reducing atmosphere. Iron ore in its crude state is of a composition corresponding to  $Fe_2O_3$ . Roasting in this manner reduces this compound to  $Fe_3O_4$  which is known as magnetic oxide of iron. This reduction of the ore from its ferric form to the form of magnetite renders it susceptible of being magnetically separated from the other constituents of the material in the roaster. If found necessary reducing agents can be employed to facilitate the reduction of the ferric oxide to magnetite.

Ore thus roasted and converted may be classified into two sizes and then concentrated by means of magnetic cobbers and/or magnetic log washers. The first of these machines mentioned, namely, the magnetic cobbers, are adapted to concentrate the large size which is substantially over 100 mesh while the magnetic log washers concentrate the small size of less than 100 mesh. It will be appreciated that the tailings from the magnetic concentrating machines will be extremely low in iron content and may economically be passed to waste.

If desired the tailings from the grizzly, the screen 3, the log washer 8, and the Dorr bowl classifier may be treated in a manner similar to that just described in connection with the jig and Rheolaveur machine tailings. Prior to such treatment of these tailings, however, it will be necessary to reduce the ore by crushing to a suitable size whereby the magnetic separation may be effected. In any event the tailings thus treated instead of being wasted as discards are treated in an economical and practical manner to place them in condition for use in the blast furnace.

In lieu of magnetic treatment, there might possibly be substituted further tabling. From the foregoing description it will be appreciated that a mineral separation process which does not exceed the economic limit heretofore referred to and which results in a maximum yield of concentrates possessing an extremely low percentage of impurities has been devised. As evidence of this, attention is called to Table III compiled from analyses kept at the Harrison washing plant, previously mentioned.

TABLE III  
Total concentrate analysis of the Harrison washing plant

| Treatment of concentrates | Tonnage percentage | Percentage composition of major constituents of the ore |                |
|---------------------------|--------------------|---------------------------------------------------------|----------------|
|                           |                    | Iron                                                    | Silica         |
| Not jigged or Rheo'd      | 50.00              | 55.51<br>53.85                                          | 14.39<br>17.03 |
| Jigged and Rheo'd         | 39.95              | 58.42<br>56.95                                          | 10.23<br>12.00 |

In both sets of values given in Table III the log washer concentrates were neither jigged nor subjected to the second washing stage, but were mixed directly with the total jig and the total Rheolaveur concentrates. However these figures will adequately show the advantageous effects of employing the jigging step and the second washing step. It may be observed that when the two maximum values of the iron percentages are compared there will be found an increase in the iron content of substantially 3% when the jigging and second washing step are employed while the silica values associated with those of the iron show a decrease in the silica content of over 4%. The same holds true for the sets of minimum values where the increase in the iron content is substantially 3% and the decrease in the silica content is over 5%.

It will be appreciated that when the tailings from the second washing step and from the jigs are treated as herein set forth to convert the same into magnetic iron oxide and then separate the magnetic iron oxide from the bulk of the material, the efficiency of the process can be greatly improved.

While in disclosing the foregoing process and its modifications, reference has been made to a specific crude ore and to specific concentrations of iron and silica in the ore, it is to be clearly understood that iron ore containing a varying iron

and silica content may be treated to advantage in accordance with the present invention. Ores containing other constituents may be advantageously treated by the processing described. It is also to be understood that while in describing the operation of the present invention, reference has been made to specific types of concentrating, washing, crushing and other ore conditioning apparatus and to specific sizes of the ore conditioned, that other machines susceptible of carrying out the several steps as herein set forth may be employed to advantage. Likewise, the ore undergoing treatment may be conditioned as to sizes other than those herein set forth.

While there has been shown and described the preferred embodiment of my invention, it is to be understood that the invention is not confined to the precise details of construction herein set forth, by way of illustration, as it is apparent that many changes and variations may be made therein by those skilled in the art without departing from the spirit of the invention, or exceeding the scope of the appended claims.

We claim:

1. A process for conditioning iron ore, comprising progressively sizing the ore into decreasing sizes, further sizing the oversized last obtained and jigging in separate lots the products of the last mentioned sizing, passing the undersized of the first mentioned sizing to a log washer, treating the overflow from the washer in a bowl classifier, passing the concentrates from the washer and classifier to a launder type classifier, and collecting the concentrates of the last mentioned classifier and the jigging.

2. A process for conditioning iron ore, comprising progressively sizing the ore into decreasing sizes, treating the fines last obtained from said sizing in a log washer, combining the washer concentrates and the last over-size from the sizing, sizing such combined material and jigging the resulting sizes separately, and passing the tails from the log washer to a bowl classifier.

3. A process for conditioning iron ore, comprising progressively sizing the ore into decreasing sizes, treating the fines last obtained from said sizing in a log washer, combining the washer concentrates and the last oversize from the sizing, sizing such combined material and jigging the resulting sizes separately, passing the tailings from the log washer to a bowl classifier, and subjecting the concentrates from such bowl classifier to treatment in a launder type classifier.

EMMETT BUTLER.

ARTHUR K. KNICKERBOCKER.

RICHARD O. HOCKING.

60

65

70

75

80

85

90

95

100

105

110

115

120

125

135

140

145

150